# EUROPEAN PATENT SPECIFICATION

(11) **EP 1 444 371 B1**
(45) Date of publication and mention of the grant of the patent: **13.04.2005**
(21) Application number: 02793320.9
(22) Date of filing: 15.11.2002
(51) Int. Cl.: C21D 8/02, C21D 9/52

(54) **IN-LINE PROCESS FOR THE RECRYSTALLIZATION OF SOLIDIFIED COARSE STRIPS IN CARBON STEEL AND IN LOW-ALLOYED STEEL**
IN-LINE-VERFAHREN ZUM REKRISTALLISIEREN VON ERSTARRTEN GROBBÄNDERN IN UNLEGIERTEM STAHL UND NIEDRIG LEGIERTEM STAHL
PROCEDE EN LIGNE POUR LA RECRISTALLISATION DE BANDES BRUTES SOLIDIFIEES EN ACIER AU CARBONE ET EN ACIER FAIBLEMENT ALLIE

(30) Priority: 15.11.2001 IT RM20010678
(43) Date of publication of application: 11.08.2004
(73) Proprietor: Thyssenkrupp Acciai Speciali Terni S.p.A., 05100 Terni (IT)
(72) Inventor: ANELLI, Ettore, Centro Svilupp Materiali S.p.A., I-00129 Roma (IT); PORCU, Giorgio, Centro Sviluppo Materiali S.p.A., I-00129 Rome (IT); SARTINI, Luca, ThyssenKrupp Acciai Speciali Terni, I-05100 Terni (IT)
(74) Representative: Leone, Mario
(86) International application number: PCT/IT2002/000728
(87) International publication number: WO 2003/062476

(56) References cited:
- EP-A- 0 707 908
- EP-A- 0 776 984
- EP-A- 0 818 545

## Description

The present invention applies to both Carbon and low-alloyed steel strips, made by direct continuous casting with a twin-roll strip machine, all characterized by the generation of large-size grains (from 150 to 1500 µm) in the solidified coarse product.

The invention refers to an in-line controlled recrystallization treatment carried out on a solidified coarse strip during its roll path transfer, prior to its wrapping on a coiler. In particular, there are carried out in-line and in rapid succession a rolling and an annealing (rapid heating with holding at preset temperatures for short times) so as to attain a practically complete recrystallization of the austenite or of the other microstructural components (e.g., ferrite) work hardened in the preceding deformation. Both the rolling and the annealing can be carried out under conditions in which the austenite or the ferrite are stable, or in a mixed-phase field, in which both the austenite and the ferrite are stable.

This invention refers to a process for the making of steel strips and sheets, having a thickness ranging from 4.5 to 0.7 mm, corresponding to common- or special-type hot-rolled or cold-rolled and annealed products, using as starting material continuous casting coarse strips and the present in-line recrystallization process.

Several processes for improving the mechanical properties of continuously cast strips via the homogenizing and the refining of the primitive austenitic grains by thermomechanical treatments have already been advanced and patented.

In particular, EP 0707908 Al teaches a twin-roll continuous casting apparatus with which a Carbon steel strip is cast under an atmosphere of inert gas, like Ar or N₂. The strip is then subjected in-line to hot rolling(from 850 to 1350 °C) with a thickness reduction ranging from 5 to 50% and cooled. The thin flat product thus obtained has good strength and ductility properties by virtue of the grain size reduction attained by hot rolling.

Other structure refining methods (JP 61689846 and JP 63115654) refer to in-line thermal treatments, without hot rolling, comprising at least a double phase transition prior to the final cooling and wrapping. Said phase transition is effected subjecting the strip to single or multiple heat cycles of the type: cooling, heating, cooling. With specific reference to Carbon steel and low-alloyed steel in a cast coarse product state, in EP 0707908, EP 0818545 and JP 3249126 the processes and the apparatuses for carrying out in-line thermal treatments are described in which, prior to or after the optional hot reduction of the thickness of the cast coarse strip, a cooling and a subsequent in-furnace heating of the strip is carried out, aimed at refining the structure through the nucleation mechanism of new austenitic grains after phase transformation in the ferritic field. Some of the above reported processes are aimed, besides at refining the structure in order to improve mechanical characteristics like strength, ductility and toughness, at attaining an adequate surface finishing of the strip (roughness).

Also WO 95/13155 (ISHIKAWAJIMA and BHP) teaches an in-line thermal treatment of cast Carbon steel strip aimed at checking the microstructure of the as-cast strip. In particular, the cast strip, after an optional single-pass thickness reduction (20-50%) at 900-1100 °C, is cooled below the temperature at which the transformation of austenite into ferrite takes place, and subsequently heated in-furnace at <1200°C temperatures until reaustenizing the material (in-line normalization). The austenitic grains are thus refined, and, by checking the strip final cooling and wrapping, sufficiently refined structures providing adequate strength and ductility can be developed.

EP 0776984 (Nippon Steel) reports a method and the related equipment for continuously manufacturing metal coils, from a continuous casting system of strips, comprising also the steps of: hot deformation, with a >30% thickness reduction; in-furnace heating thermal treatment under non-oxidizing atmosphere at temperatures of 800-1250 °C (preferably of 1100-1250 °C); cooling, at a 20-40 °C/s rate and down to 100 °C; pickling; and strip wrapping/shearing. The main object of this invention is the connection between the main casting line and the strip pickling-edge trimming-end thermal treatment line, so as to carry out a single continuous step according to which the pickling, the edge trimming, the strip wrapping/shearing lines may independently be connected to the strip casting-rolling-thermal treatment line. The sole example reported relates to a stainless steel, although the metals usable in the invention comprise common and special steels.

Also EP 0760397 (Nippon Steel) discloses an apparatus for stainless steelmaking realizing a process comprising the steps of: casting, cooling, hot deformation (rolling) at various temperatures, complete recrystallization by heating and cooling.

Some of the above processes and other alike ones require the introduction of one or more optional cooling systems and of a rolling stand, as well as of an intermediate reheat furnace, located upstream or downstream of the rolling stand onto the roll path transferring the strip to the coiler.

Most of the preceding experiences with Carbon steel and low-alloyed steel relate to in-line thermal or thermomechanical treatments exploiting sequential phase transformations of the austenite-ferrite-austenite type to attain, prior to the cooling preceding the strip wrapping, a homogenizing and a refining of the austenitic structure, so as to make it as similar as possible to that of a conventionally hot-rolled strip.

The state of the art provides no teachings about the attainment of a Carbon steel or low-alloyed steel product that, from a continuously cast solidified coarse strip, develop the desired mechanical and technological properties, related to hot-rolled or cold-rolled and annealed strips and sheets, exploiting a controlled in-line recrystallization treatment, by rolling in a ferritic, austenitic or mixed-phase field, and direct annealing, also in a subcritical field (<Ac₃ in-furnace treatment temperature).

The few occurrences of in-line recrystallization refer to high-alloyed (stainless) steels that always recrystallize at a very slow rate, as much so as to systematically require treatment temperatures of well above 1050 °C in order to attain a significant recrystallization over short times.

Also for Carbon steel, generally having recrystallization kinetics significantly faster than those of the stainless steels, the presence of very coarse grains in the solidified coarse strips inhibits the recrystallization process. Hence, though deforming at high temperatures the solidified strip and imposing elevated deformation in a single pass, the recrystallization is merely partial, with several grains practically conserving their initial geometry. If in the Carbon steel there are introduced also other alloy elements like Si, Cr, Ni, and/or microalloy elements like V and Nb, often required in order to attain certain mechanical properties and microstructures, the recrystallization at <950°C temperatures is practically non-existent. It has to be borne in mind that in the state-of-the-art systems the contact with the water-cooled rolls causes sensible strip cooling, also because the rolling rates are very low (elevated contact times) and the reductions imposed by single pass are often elevated (greater length of the arc of contact). Immediately post-rolling, the typical temperatures for casting coarse thin strips (<3.5 mm) are generally of <1050 °C, often of <1000 °C, dropping to <950°C within a few seconds even in case of a still-air cooling of the strip. Hence, to date in the known processes the recrystallization of cast coarse structures in Carbon steel and in low-alloyed steel is always partial, with non-homogeneous structures having mainly large-sized grains unsuitable for developing the desired end properties.

An object of the present invention is that of providing an in-line process for the making of strips in Carbon steel and in low-alloyed steel by a controlled recrystallization treatment performed on a solidified coarse strip during the roll path transfer, prior to the wrapping on the coiler.

In particular, there are carried out in-line and in rapid succession a rolling, an annealing (rapid heating with holding at preset temperatures for short times in order to attain a near-complete recrystallization of the austenite and/or of the ferrite work hardened during the deformation), and a controlled cooling (optional direct galvanizing included) prior to the wrapping on the coiler.

This object is attained by a process for the making of steel strips as defined by claim 1.

This novel process comprises the following steps:
■ casting, in a twin-roll continuous casting machine (A), of strips having a thickness ranging from 1 to 6 mm and a composition, expressed as percent by mass, comprising the following components:
   0.02-0.20 C; 0.1-1.6 Mn; 0.02-2.00 Si; <0.05 Al; <0.03 S; <0.1 P; 0.01-1.5 Cr; 0.01-0.5 Ni; <0.5 Mo; 0.003-0.012 N; and optionally, <0.03 Ti; <0.10 V; <0.035 Nb; < 0.005 B,> **rest Fe and unavoidable impurities;**
■ controlled cooling of the strip in the section comprised between the casting rolls and a rolling system (E);
■ hot deformation of the strip cast with said rolling system (E) at a temperature ranging from 1150 to (Ar₁ - 100) °C, until effecting a 15 to 80% thickness reduction thereto, said hot deformation being selected from the group comprising:
   - rolling, at >Ar₃ temperatures and in a completely austenitic phase, Ar₃ being the transformation start temperature of the continuously cooled austenite;
   - rolling, at a <Ar1 temperature and in a completely ferritic phase;
   - rolling, at temperatures ranging from Ar₃ to Ar₁ and under coexistence conditions of the austenitic phase and of the ferritic phase;
■ holding the strip at a controlled temperature in an insulated system (F) comprised between an outlet of the rolling system (E) and an inlet in a heating system (G);
■ heating the strip with said heating system (G) at temperatures ranging from 670 to 1150 °C for times ranging from 5 to 40 s, so as to attain a >95% **in volume** strip recrystallization;
■ controlled cooling in the section comprised between an outlet of said heating system (G) and a wrapping system, optionally having plural coilers (N, P), of the strip so obtained.

Another object of the present invention is to provide strips of Carbon steel and of low-alloyed steel, manufactured with the hereto detailed process, having an end thickness ranging from 4.5 to 0.7 mm and preset microstructure characteristics, capable of developing the following properties, suitable for various application fields:
■ Cold formability for non-severe applications like bending and drawing, for the manufacturing of components for electrical household appliances (e.g., caps for refrigerators, radiators, refrigerating systems) and for the building industry (e.g., gutters, window frames, garage doors, ceilings, etc.).
■ Cold forming even for severe applications (e.g., wheel rims).
■ Structural employ (e.g., guard-rail, car components, containers, etc.).

The present invention will hereinafter be better illustrated by the description of an embodiment thereof given by way of example and without limitative purposes, with the aid of the attached drawings, wherein:
* FIG. 1 is a simplified scheme of the continuous casting machine for thin strips and of the devices for the in-line recrystallization and the highly controlled cooling of the strips, used for the present invention;
* FIG. 2 is a scheme of the in-line recrystallization and of the cooling cycles applied to cast coarse strips;
* FIGGS. 3 and 4 show strip microstructures, as detectable by optical microscope.

With reference to FIG. 1, the process of the present invention provides the use of a continuous casting machine having a twin-roll ingot mold (A), all characterized by the formation of large-size grains (150 to 1500 µm) in the solidified coarse product. Directly downstream, there are provided cooling devices (B and D) for cooling in a controlled manner the strip continuously crossing them, guided by the pinch rolls (C) of a *per se* already known construction.

During the solidification and the extraction from the ingot mold (A) the strip is subjected to an adequate force, e.g. acting on the twin rolls, so as to limit the generation of shrinkage cavities. Then, the cast strip is subjected on both faces thereof to cooling in order to slow down the growth both of the austenitic grains and of the surface oxide layer. The cooling cycles of the as-cast steel strips are set acting on the casting rate, the flow rates and the number of active cooling areas (modules).

The pair of said cooling systems B and D has modules, individually actuable, variable in the individual sections and capable of effecting onto the strip cooling rates of up to 200 °C/s.

In said modules, the cooling is attained with cooling modes selected from the group comprising: natural air, forced air, inert gas jets in an inertized chamber, air-water, water and combinations thereof.

Downstream of the cooling system D there is provided a rolling system consisting of one or more stands (E), capable, in one or more passes, of effecting a 15-80% total thickness reduction in order to reduce to acceptable sizes the residual porosities due to the solid contraction and to induce a work hardening of the structure extant at the instant of deformation.

The stands are located as close as possible, so as to attain quite short interpass times (shorter than the time required to attain the 50% **in volume** recrystallization) and to allow deformation accumulation in the material (the greater the accumulated deformation, the more rapid the material recrystallization and the softening kinetics).

In particular, the hot deformation of the cast strip can take place by means of two consecutive stands, each providing a 15-40% thickness reduction.

Moreover, there is provided a rapid heating system (R), aimed at controlling the temperature of the strip inletted in the rolling system (E), according to the steel composition and to the thermomechanical cycle to be carried out.

The rapid heating system (R) is located downstream of the controlled cooling system (D).

At the outlet of E there is located a further system (F), comprising a tunnel insulated under natural air, or inert gas, or combinations thereof, and aimed at holding the temperature of the strip which is about to enter the furnace (G) located nearby E. In particular, in the case of austenitic-phase rolling, the insulated section prevents temperature from dropping below Ar₃ and to start a phase transformation before the austenite recrystallization.

The furnace (G), of an induction-, gas- or the like type, is capable of operating under a reducing or a non-oxidizing atmosphere, and of rapidly (in less than 12 s) bringing the strip temperature to temperature values ranging from 670 to 1150 °C, apt to attain a near-complete recrystallization of the material (>95 % **in volume**) with temperature holding times of 5-40 s. The annealing temperature is selected so as to fall within a completely austenitic field (austenitic field rolling) or a ferritic field (ferritic field rolling) , or within a mixed-phase field in which ferrite and austenite coexist (ferritic or mixed-phase field rolling), as it is indicated in FIG. 2.

Right at the furnace outlet there is located the cleaning system (H), which removes oxides or oxide residues partially or totally reduced by the furnace atmosphere from the strip surface.

Downstream of the system H, along the roll path leading to the coilers (N, P) there is located a set of at least three controlled cooling modules (I, L, M). These modules are capable of effecting on the strip cooling rates variable in the individual sections and ranging from 800 °C/s (ultrarapid cooling) to 0.01 °C/s (insulation).

Upon detecting the strip temperature at the furnace outlet by metering with a suitable device, the strip cooling cycle is defined according to the steel phase transformation characteristics, which mainly depend on the actual size of the austenitic grains and on the chemical analysis of the steel, so as to develop the desired structures. Onto the roll path, among the various modules, there are located other temperature meters (e.g., pyrometers), enabling monitoring of the thermal cycle. The latter can be quite complex (e.g., accelerated cooling, in-air cooling, wrapping) in case multiphase microstructures, made of various constituents like polygonal ferrite, bainite, martensite and/or residual austenite, are to be developed.

One of the cooling modules is also capable of galvanizing the strip.

However, preferably the strip is wrapped at a temperature of from 900 to 150°C.

Various laboratory and full-scale plant tests were coaducted, employing steels whose composition in percentage by mass was defined in the following field: 0.02-0.20 C; 0.1-1.6 Mn; 0.02-2.00 Si; <0.05 Al; <0.03 S; <0.1 P; 0.01-1.5 Cr; 0.01-0.5 Ni; <0.5 Mo; 0.003-0.012 N; and, optionally, <0.03 Ti; <0.10 V; <0.035 Nb; <0.005 B, **rest Fe and unavoidable impurities.**

These tests highlighted that:
a) The grains of the cast coarse strip have coarse mean sizes (>150 µm) and often a column-type shape resembling the solidification macrostructure.
b) The dynamic recrystallization, with these sizes of the initial grains and for the aboveindicated chemical analyses, is not activated for the typical in-line rolling conditions of cast coarse strips (15-40% reduction, 10-35 s⁻¹ deformation rate, 1000-1150 °C deformation temperature).
c) A 30-40% reduction at 1000-1150 °C induces a static, yet partial, recrystallization, there remaining a significant coarse grain fraction (>50% **in volume**). In fact, the austenite recrystallization kinetics, already intrinsically slow, become slower with the dropping of the strip temperature just after the end of the hot rolling. A microstructural nonuniformity ensues, which cannot be compensated acting on the subsequent checked/controlled cooling and wrapping.
d) By lowering the deformation temperature in the austenitic field the static recrystallization is inhibited, and in the subsequent phase transformation, besides at the edges of the primitive austenitic grains, ferrite nucleation ensues at the deformation bands inside of the coarse grains. The end result is a certain, yet nonhomogeneous, refining of the structure.
e) The grains located near the surfaces of the cast and rolled coarse strip are often thinner than those at midthickness, due to the dishomogeneity of thickness deformation and of temperature gradients in the in-line rolling.
f) The missed or incomplete recrystallization after the in-line rolling, combined to the scanty refining and to the low uniformity of the resulting microstructure, is a critical factor for the development of strips for structural employ (requiring high strength and adequate toughness) and for direct application, replacing the cold-rolled strips used in the building and household appliance fields.
g) A near-complete recrystallization (>95% **in volume**) of the austenite having a very coarse initial structure is attained in less than 40 s even in low-alloyed steel having a composition which falls within the indicated limits, introducing an in-line annealing, at 1050-1100 °C temperatures, immediately after the hot rolling stage (>15% deformation at 950-1150 °C).
h) Much higher temperatures, do accelerate the static recrystallization, leading however to overly large sizes (>120 µm) of the recrystallized austenitic grains.
i) After the in-line controlled recrystallization treatment, the austenitic grains are equiaxic and uniform, with mean sizes ranging from 50 to 120 µm, according to the deformation accumulated in rolling and at the annealing temperatures adopted. These austenitic grains, after the checked cooling, generate ferritic grains having 15-30 µm sizes, in case of >10 °C/s cooling rates and of wrappings at >700 °C temperatures. In the latter case, also pearlite islands are observable whose volume fraction relates to the Carbon content in the steel.
j) The in-line recrystallization allows, by homogenizing the austenitic structure and the strip temperatures lengthwise as well as widthwise, to reduce the variety of structures, polygonal, acicular and otherwise unavoidable, entailing advantages of reproducibility of the mechanical characteristics, in particular for the direct-employ products, replacing the traditional cold-annealed strips.
k) The rolling of the cast coarse strip, in the case of low-Carbon strips (C <0.06 %), may be carried out without the problem of excessive rolling forces even in the ferritic field, i.e. at temperatures ranging from Ar₁ to Ar₁ - 100°C. For >25 % deformations in the ferritic field and in-line annealing conducted at a 670-720 °C temperatures, always for <40 s times, with rapid wrapping of the strip at such temperatures, ferrite structures with grains or subgrains having 30-60 µm sizes (low yield value) and a homogeneous carbide distribution (absence of lamellar pearlite) are obtained, suitable for nonsevere cold forming steps, like bending and drawing.

In case of rolling in a ferritic or mixed-phase field, even 0.06 - 0.2% Carbon steel strips can be annealed over short times. In this case, a subcritical field (Ac₁ - Ac₃) annealing is resorted to. The temperature is set according to the quantity of austenite in the strip and to the desired Carbon enrichment of the latter at the furnace outlet, prior to the controlled cooling which is modulated according to the desired quantities and typologies of the end structures dispersed in the extant ferrite (e.g., bainite and high-Carbon martensite islands, or bainite and residual austenite islands).

The present innovative in-line recrystallization treatment of cast coarse strips enables, by selecting the chemical analysis of the steel, to check the rolling and annealing temperatures and the in-line cooling cycles, to develop suitable end microstructures, having definite volume fractions of equiaxic (polygonal) ferrite, pearlite or carbides, of acicular and/or bainitic ferrite and of high-Carbon martensite/residual austenite islands. The different distribution of the microstructural components so obtained, highly checkable through the thermal and microstructural homogenization taking place during the in-furnace recrystallization treatment, provides the strips with different combinations of strength, ductility and cold formability.

In particular, there were evaluated the properties related to the generation of ferrite structures having a 30-80 µm equiaxic grain and pearlite or nonlamellar carbides, obtained by in-line recrystallization of the austenite or of the ferrite, respectively, deriving from cast coarse strips, in low-Carbon (C <0.06 %) steels having a very coarse primitive structure.

Treatments for the in-line recrystallization and the controlled cooling of the cast coarse strips in low-alloyed steel, containing Mn, Si and optionally other elements like Cr, were carried out in order to develop multiphase structures containing ferrite (>55%), bainite (5-40%), and a scattering of high-Carbon (1-15% C) martensite islands. The latter are characterized by having, at the ferrite interface, a high dislocation density with respect to the traditional polygonal ferrite/pearlite structures.

The end material yielded has a continuous-type stress-deformation curve, provided with a good mix of strength and ductility. Exploiting a subcritical recrystallization treatment in continuously cast strips, microstructures exhibiting significant quantities of residual austenite (5-20 %) were made.

According to the object of the present invention, hereinafter some embodiments thereof are disclosed.

### EXAMPLE 1

An 1.6 mm thickness strip was made according to the process of the present invention and using steel A, the analysis of the latter being reported in Table 1.

**Table 1**

| **Chemical analysis of steel A** | | | | | | | | | | | | |
|---|---|---|---|---|---|---|---|---|---|---|---|---|
| Steel | C | Mn | Si | Cr | Ni | Cu | Ti | Mo | S | P | Al | N |
| A | 0.048 | 0.73 | 0.28 | 0.07 | 0.07 | 0.18 | 0.01 | 0.02 | 0.002 | 0.008 | 0.005 | 0.0065 |

The molten steel was cast in a vertical continuous casting machine (Fig. 1) having a twin-roll ingot mold and a 6 t/m mean separation force. The strips were cooled at the ingot mold outlet until reaching a 1080-1100 °C temperature at the rolling system inlet. A 35% total thickness reduction was effected. The subsequent cooling and heating steps were carried out as it is schematically shown in FIG 2, so as to attain a ≥ 850 °C minimum temperature Tm, a 10 °C/s heating rate, a 1050 °C maximum temperature of the in-furnace strip, with 10 s holding times thereat. 15 °C/s cooling rates were detected at the furnace outlet and up to the wrapping. The latter was carried out at >750 °C temperatures. The microstructural characteristics and the mechanical properties of the end strip, in terms of mean size (d) of the ferrite grains, pearlite (P) %, lowest yield value (Re_{L}), failure strength (Rm), Re_{L}/Rm ratio, ultimate elongation (A), are reported in Table 2. The ratio between the standard deviation and the mean value for the failure strength and for the elongation is of the 2.5% and of the 3%, respectively. These values indicate a high checkability of the end microstructure, induced by the introduction of the in-line recrystallization.

**Table 2**

| **Microstructural characteristics and mechanical properties of the 1.6 mm end thickness A steel strip** | | | | | |
|---|---|---|---|---|---|
| d (□m) | P (%) | ReL (MPa) | Rm (MPa) | Rs/Rm (-) | A (%) |
| 17 | 2 | 260 | 365 | 0.71 | 28 |

FIG. 3 shows the typical microstructure of the strip, as observable at the optical microscope.

Apparently, a ferrite structure having equiaxic-grain and pearlite islands was generated.

### EXAMPLE 2

An 1.6 mm end thickness strip was made according to the process of the present invention and using steel B. The analysis of the latter is reported in Table 3.

**Table 3**

| **Chemical analysis of steel B** | | | | | | | | | | | | |
|---|---|---|---|---|---|---|---|---|---|---|---|---|
| Steel | C | Mn | Si | Cr | Ni | Cu | Ti | Mo | S | P | Al | N |
| B | 0.11 | 0.80 | 0.29 | 0.06 | 0.04 | 0.05 | 0.005 | 0.01 | 0.003 | 0.007 | 0.027 | 0.0042 |

The molten steel was cast in a vertical continuous casting machine having a twin-roll ingot mold and a 5.5 t/m mean separation force. The strips were cooled at the ingot mold outlet until reaching a 1080-1100 °C temperature at the rolling system inlet. A 35% total thickness reduction was effected. The subsequent cooling and heating steps were carried out as it is schematically shown in FIG. 2, so as to attain a ≥850 °C minimum temperature Tm, an 8 °C/s heating rate, a 1050 °C maximum temperature of the in-furnace strip, with 12 s holding times thereat. 15 °C/s cooling rates were detected at the furnace outlet and up to the wrapping. The latter was carried out at >750 °C temperatures. The microstructural characteristics and the mechanical properties of the end strip, in terms of mean size (d) of the ferrite grains, pearlite % (P) lowest yield value (Re_{L}), failure strength (Rm), Re_{L}/Rm ratio, ultimate elongation (A), are reported in Table 4. The ratio between the standard deviation and the mean value for the failure strength is of the 3% and of the 3.5%, respectively.

**Table 4**

| **Microstructural characteristics and mechanical properties of the 1.6 mm end thickness B steel strip** | | | | | |
|---|---|---|---|---|---|
| d (□m) | P (%) | ReL (MPa) | Rm (MPa) | Rs/Rm (-) | A (%) |
| 14 | 10 | 270 | 390 | 0.69 | 24 |

FIG. 4 shows the typical microstructure of the strip, as observable at the optical microscope.

### EXAMPLE 3

An 1.6 mm thickness strip was made, according to the process of the present invention and using steel A. The analysis of the latter is reported in Table 1.

The molten steel was cast in a vertical continuous casting machine having a twin-roll ingot mold and a 6 t/m mean separation force. The strips were cooled at the ingot mold outlet until reaching a 690 °C temperature at the rolling system inlet. A 37% total thickness reduction was effected. The subsequent cooling and heating steps were carried out as it is schematically shown in FIG. 2, so as to attain a ≥670 °C minimum temperature Tm 670 °C, a 5 °C/s heating rate, a 720 °C maximum temperature of the in-furnace strip, with 15 s holding times thereat.
<0.5 °C/s cooling rates were detected at the furnace outlet and up to the wrapping.

The latter was carried out at ≥ 700 °C temperatures. The microstructural characteristics and the mechanical properties of the end strip, in terms of mean size (d) of the ferrite grains, lowest yield value (Re_{L}), failure strength (Rm), Re_{L}/Rm ratio, ultimate elongation (A), are reported in Table 5.

**Table 5**

| **Microstructural characteristics and mechanical properties of the 1.6 mm end thickness in-line recrystallized, ferritic-phase rolled A steel strip** | | | | |
|---|---|---|---|---|
| d (□m) | ReL (MPa) | Rm (MPa) | Rs/Rm (-) | A (%) |
| 30 | 370 | 450 | 0.82 | 32 |

Optical microscope observation highlighted a ferrite structure having dispersed nonlamellar carbides onto the strip so obtained.

### EXAMPLE 4

A 2.4 mm end thickness strip was made, according to the process of the present invention and using steel C. The analysis of the latter is reported in Table 6.

**Table 6**

| **Chemical analysis of steel C** | | | | | | | | | | | | |
|---|---|---|---|---|---|---|---|---|---|---|---|---|
| Steel | C | Mn | Si | Cr | Ni | Cu | Ti | Mo | S | P | Al | N |
| C | 0.15 | 1.55 | 1.42 | 0.10 | 0.05 | 0.1 | 0.005 | 0.02 | 0.005 | 0.092 | 0.03 | 0.054 |

The molten steel was cast in a vertical continuous casting machine having a twin-roll ingot mold and a 6.5 t/m mean separation force. The strips were cooled at the ingot mold outlet and then heated until reaching an 840-860 °C temperature at the rolling system inlet. A 40% total thickness reduction was effected. The subsequent cooling and heating steps were carried out as it is schematically shown in FIG. 2, so as to attain a ≥880 °C minimum temperature Tm, an 8 °C/s heating rate, a 1050 °C maximum temperature of the in-furnace strip, with 12 s holding times thereat. Downstream of the furnace the cooling rates were of from 50 °C/s to 700-680 °C/s, 5 s natural air cooling, ≤400 °C forced cooling (40-80 °C/s).

### Wrapping at 400-380 °C temperatures

A mixed ferrite/bainite structure having residual austenite islands was generated. The percent by volume of residual austenite, measured by X-ray diffraction, was of the 12%. This structure confers the mechanical properties shown in Table 7.

**Table 7**

| **Microstructural characteristics and mechanical properties of the 2.2 mm end thickness C steel strip** | | | | |
|---|---|---|---|---|
| Austenite (%) | Rp0.2 (MPa) | Rm (MPa) | Rs/Rm (-) | A (%) |
| 12 | 570 | 980 | 0.57 | 24 |

The elevated yield value (Rp_{0.2} ) and failure strength value Rm are anyhow accompanied by a low yield/failure ratio, a good ductility (>22% elongation), and a particularly high (>16000 MPa%) product of the elongation X failure strength (A X Rm) parameter.

These characteristics are conferred by the good structural homogeneity and by the presence of residual austenite, attained with the in-line recrystallization of continuous casting coarse strips.

## Claims

1. A process for the making of strips in Carbon steel and in low-alloyed steel having a highly checked microstructure, comprising in sequence the following steps:
■ casting, in a twin-roll continuous casting machine (A), of strips having a thickness ranging from 1 to 6 mm and a composition, expressed as percent by mass, comprising the following components:
0.02-0.20 C; 0.1-1.6 Mn; 0.02-2.00 Si; <0.05 Al; <0.03 S; <0.1 P; 0.01-1.5 Cr; 0.01-0.5 Ni; <0.5 Mo; 0.003-0.012 N; and, optionally, <0.03 Ti; <0.10 V; <0.035 Nb; < 0.005 B,> **rest Fe and unavoidable impurities;**
■ controlled cooling of the strip in the section comprised between the casting rolls and a rolling system (E);
■ hot deformation of the cast strip by said rolling system (E) at a temperature ranging from 1150 to (Ar₁ - 100) °C, until effecting a 15 to 80% thickness reduction thereto, said hot deformation being selected from the group comprising:
- rolling, at >Ar₃ temperatures and in a completely austenitic phase, Ar₃ being the transformation start temperature of the continuously cooled austenite;
- rolling, at a <Ar₁ temperature and in a completely ferritic phase;
- rolling, at temperatures ranging from Ar₃ to Ar₁ and under coexistence conditions of the austenitic phase and of the ferritic phase;
■ holding the strip at a controlled temperature in an insulated system (F) comprised between an outlet of the rolling system (E) and an inlet in a heating system (G);
■ heating the strip with said heating system (G) at temperatures ranging from 670 to 1150 °C for times ranging from 5 to 40 s, so as to attain a >95 % **in volume** strip recrystallization;
■ controlled cooling in the section comprised between an outlet of said heating system (G) and a wrapping system, optionally having plural coilers (N, P), of the strip so obtained.

2. The process for the making of strips in Carbon steel and in low-alloyed steel according to claim 1, **wherein, in said casting step** the composition of said strip **also comprises:** <0.03 Ti; <0.10 V; <0.035 Nb and <0.005 B.

3. The process for the making of strips in Carbon steel and in low-alloyed steel according to claim 1 or 2, wherein said controlled cooling in the section comprised between the casting rolls and the pinch-rolls C, and between the pinch rolls (C) and the rolling system (E) takes place by means of a pair of systems (B and D), having modules, individually acbuable, variable in the individual sections and capable of effecting onto the strip cooling rates of up to 200 °C/s.

4. The process for the making of strips in Carbon steel and in low-alloyed steel according to claim 3, wherein said cooling is attained with cooling modes selected from the group comprising: natural air, forced air, inert gas jets in an inertized chamber, air-water, water and combinations thereof.

5. The process for the making of strips in Carbon steel and in low-alloyed steel according to any one of the claims 1 to 4, wherein said heating system (G) operates under a reducing or a non-oxidizing atmosphere.

6. The process for the making of strips in Carbon steel and in low-alloyed steel according to claim 5, wherein said heating system (G) operates at temperatures selected from the group comprising: temperatures corresponding to that of the existence of the sole austenitic phase, temperatures corresponding to that of the existence of the sole ferritic phase, temperatures corresponding to that of coexistence of the ferritic and of the austenitic phase.

7. The process for the making of strips in Carbon steel and in low-alloyed steel according to claim 6, wherein said heating system (G) is followed by a system (H) for cleaning the strip surface and for removing therefrom oxides or oxide residues partially or totally reduced by the furnace atmosphere.

8. The process for the making of strips in Carbon steel and in low-alloyed steel according to any one of the claims 1 to 7, wherein the strip is held at a controlled temperature at the outlet of the rolling system (E) by a system (F) comprising an insulated tunnel containing air, or inert gas, or combinations thereof.

9. The process for the making of strips in Carbon steel and in low-alloyed steel according to any one of the claims 1 to 8, wherein at the outlet of the heating system (G) the strip is subjected to a cooling with at least three modules (I, L, M), located along a roll path, capable of effecting on the strip cooling rates variable in the individual sections and ranging from 800 °C/s to 0.01 °C/s.

10. The process for the making of strips in Carbon steel and in low-alloyed steel according to **claim 9,** wherein in one of said at least three (I,L,M) modules a strip galvanizing can be carried out.

11. The process for the making of strips in Carbon steel and in low-alloyed steel according to any one of the preceding claims, wherein the hot deformation of the cast strip takes place by means of two consecutive stands, each providing a 15-40% thickness reduction.

12. The process for the making of strips in Carbon steel and in low-alloyed steel according **to claim 11,** wherein the interpass time between consecutive stands is shorter than the time required to attain a 50% **in volume** recrystallization.

13. The process for the making of strips in Carbon steel and in low-alloyed steel according to claim 3, wherein there is provided a system (R) for heating the strip in the section comprised between the pinch rolls (C) and the rolling system (E).

14. The process for the making of strips in Carbon steel and in low-alloyed steel according to claim 13, wherein said heating system (R) is located downstream of the controlled cooling system (D).

15. The process for the making of strips in Carbon steel and in low-alloyed steel according to any one of the preceding claims, wherein the strip is wrapped at temperatures ranging from 150 to 900 °C.

## Patentansprüche

1. Verfahren zur Herstellung von Streifen bzw. Bändern aus Kohlenstoffstahl bzw. unlegiertem Stahl und aus niedrig legiertem Stahl mit einem stark überprüften Mirkogefüge, umfassend die folgenden Schritte in dieser Reihenfolge:
• Gießen von Streifen bzw. Bändern in einer kontinuierlichen Doppelwalzen-Gießvorrichtung (twin-roll continuous casting machine) mit einer Dicke in dem Bereich von 1 bis 6 mm und mit einer Zusammensetzung, ausgedrückt als Masse-%, umfassend die folgenden Bestandteile:
0,02-0,20 C; 0,1-1,6 Mn; 0,02-2,00 Si; <0,05 Al; <0,03 S, <0,1 P; 0,01-1,5 Cr; 0,01-0,5 Ni; <0,5 Mo; 0,003-0,012 N; und gegebenenfalls <0,03 Ti; <0,01 V; <0,035 Nb; <0,005 B; Rest Fe und unvermeidbare Verunreinigungen;
• Geregeltes Abkühlen des Streifens bzw. Bandes in dem Bereich, welcher zwischen den Gusswalzen und einer Walzenanlage (E) vorhanden ist,
• Heißumformen des gegossenen Streifens bzw. Bandes durch die Walzenanlage (E) bei einer Temperatur in dem Bereich von 1150°C bis (Ar₁ - 100)°C , bis daran eine Dickeverringerung von 15 bis 80% bewirkt wurde, wobei das Heißumformen aus der Gruppe gewählt wird, umfassend:
- Walzen bei > Ar₃ Temperaturen und in einer vollständig austenitischen Phase, wobei Ar₃ die Temperatur ist, bei welcher die Umwandlung des kontinuierlich abgekühlten Austenits beginnt;
- Walzen bei einer < Ar₁ Temperatur und in einer vollständig ferritischen Phase;
- Walzen bei einer Temperatur in dem Bereich zwischen Ar₃ bis Ar₁ und unter koexistierenden Bedingungen der austenitischen Phase und der ferritischen Phase;
• Halten des Streifens bzw. Bandes auf einer geregelten Temperatur in einer isolierten Anlage (F), welches zwischen einem Auslaß der Walzenanlage (E) und einem Einlass einer Heizanlage(G) vorhanden ist;
• Erwärmen des Streifens bzw. Bandes mit der Heizanlage (G) bei Temperaturen in dem Bereich von 670°C bis 1150°C für Zeiträume zwischen 5 bis 40 Sekunden, um so eine Rekristallisation von >95% bezüglich des Volumens des Streifens bzw. Bandes zu erzielen;
• Geregeltes Abkühlen des so erhaltenen Streifens bzw. Bandes in dem Bereich, welcher zwischen einem Auslaß der Heizanlage (G) und einer Einwickelanlage enthalten ist, gegebenenfalls mit einer Vielzahl von Wickelvorrichtungen (N,P).

2. Verfahren zur Herstellung von Streifen bzw. Bändern aus Kohlenstoffstahl bzw. unlegiertem Stahl und aus niedrig legiertem Stahl nach Anspruch 1, wobei die Zusammensetzung während des Gießschrittes auch umfasst: <0,03 Ti; <0,10 V; <0,035 Nb und >0,005 B.

3. Verfahren zur Herstellung von Streifen bzw. Bändern aus Kohlenstoffstahl bzw. unlegiertem Stahl und aus niedrig legiertem Stahl nach Anspruch 1 oder 2, wobei das geregelte Abkühlen in dem Bereich, welcher zwischen den Gusswalzen und den Andruckwalzen C und zwischen den Andruckwalzen (C) und der Walzenanlage vorhanden ist, mittels eines Anlagepaares (B und D) durchgeführt wird, mit Komponenten, die einzelnd betätigbar sind, und in den einzelnen Bereichen variierbar sind und in der Lage sind, auf den Streifen bzw. das Band Abkühlgeschwindigkeiten von bis zu 200°C/Sekunde auszuüben.

4. Verfahren zur Herstellung von Streifen bzw. Bändern aus Kohlenstoffstahl bzw. unlegiertem Stahl und aus niedrig legiertem Stahl nach Anspruch 3, wobei das Abkühlen durch Abkühlarten erzielt wird, gewählt aus der Gruppe umfassend: natürliche Luft, Druckluft, Schutzgasdüsen in einer inertisierten Kammer und deren Kombinationen.

5. Verfahren zur Herstellung von Streifen bzw. Bändern aus Kohlenstoffstahl bzw. unlegiertem Stahl und aus niedrig legiertem Stahl nach einem der Ansprüche 1 bis 4, wobei die Heizanlage unter einer reduzierenden oder einer nicht-oxidierenden Atmosphäre betrieben wird.

6. Verfahren zur Herstellung von Streifen bzw. Bändern aus Kohlenstoffstahl bzw. unlegiertem Stahl und aus niedrig legiertem Stahl nach Anspruch 5, wobei die Heizanlage (G) bei Temperaturen betrieben wird, ausgewählt aus der Gruppe umfassend: Temperaturen, welche dem Vorhandensein der alleinigen Austenitphase entspricht, Temperaturen, welche dem Vorhandensein der alleinigen Ferritphase entspricht, Temperaturen, welche dem Vorhandensein einer Koexistenz der Ferritphase und der Austenitphase entspricht.

7. Verfahren zur Herstellung von Streifen bzw. Bändern aus Kohlenstoffstahl bzw. unlegiertem Stahl und aus niedrig legiertem Stahl nach Anspruch 1, wobei die Heizanlage (G) von. einer Anlage (H) zur Reinigung der Streifen- bzw. Bandoberfläche und zur Entfernung von Oxiden und Oxidrückständen gefolgt wird, welche teilweise oder vollständig von der Ofenatmosphäre reduziert sind.

8. Verfahren zur Herstellung von Streifen bzw. Bändern aus Kohlenstoffstahl bzw. unlegiertem Stahl und aus niedrig legiertem Stahl nach einem der Ansprüche 1 bis 7, wobei der Streifen bzw. das Band auf einer geregelten Temperatur an dem Auslaß der Walzenanlage (E) durch eine Anlage (F) gehalten wird, umfassend einen isolierten Tunnel, welcher Luft oder Schutzgas oder deren Kombinationen enthält.

9. Verfahren zur Herstellung von Streifen bzw. Bändern aus Kohlenstoffstahl bzw. unlegiertem Stahl und aus niedrig legiertem Stahl nach einem der Ansprüche 1 bis 8, wobei der Streifen bzw. das Band an dem Auslaß der Heizanlage (H) einem Abkühlen mit wenigstens drei Komponenten (I, L, M) unterworfen wird, welche entlang einer Walzbahn angeordnet sind, die geeignet sind auf den Streifen bzw. das Band Abkühlgeschwindigkeiten auszuüben, welche in dem Bereich von 800°C/Sekunde bis 0,01 °C/Sekunde liegen.

10. Verfahren zur Herstellung von Streifen bzw. Bändern aus Kohlenstoffstahl bzw. unlegiertem Stahl und aus niedrig legiertem Stahl nach Anspruch 9, wobei in einem der wenigstens drei (I, L, M) Komponenten ein Galvanisieren des Streifens bzw. Bandes durchgeführt werden kann.

11. Verfahren zur Herstellung von Streifen bzw. Bändern aus Kohlenstoffstahl bzw. unlegiertem Stahl und aus niedrig legiertem Stahl nach einem der vorangehenden Ansprüchen, wobei die Warmumformung der gegossenen Streifen bzw. Bänder mittels zweier aufeinanderfolgender Walzgerüste durchgeführt wird, welche jeweils eine Dickeverringerung von 15-40% bereitstellen.

12. Verfahren zur Herstellung von Streifen bzw. Bändern aus Kohlenstoffstahl bzw. unlegiertem Stahl und aus niedrig legiertem Stahl nach Anspruch 11, wobei eine Durchlaufzeit zwischen den aufeinanderfolgenden Walzgerüsten kürzer ist als die Dauer um eine Rekristallisation von 50% bezüglich des Volumens zu erzielen.

13. Verfahren zur Herstellung von Streifen bzw. Bändern aus Kohlenstoffstahl bzw. unlegiertem Stahl und aus niedrig legiertem Stahl nach Anspruch 3, wobei eine Anlage (R) zur Erwärmung des Streifens bzw. Bandes in dem Bereich durchgeführt wird, welcher zwischen den Andruckwalzen (C) und der Walzenanlage vorhanden ist.

14. Verfahren zur Herstellung von Streifen bzw. Bändern aus Kohlenstoffstahl bzw. unlegiertem Stahl und aus niedrig legiertem Stahl nach Anspruch 13, wobei die Heizanlage (R) stromabwärts der geregelten Abkühlanlage (D) angeordnet ist.

15. Verfahren zur Herstellung von Streifen bzw. Bändern aus Kohlenstoffstahl bzw. unlegiertem Stahl und aus niedrig legiertem Stahl nach einem der vorangehenden Ansprüche, wobei der Streifen bzw. das Band bei Temperaturen in dem Bereich von 150 bis 900°C eingewickelt wird.

## Revendications

1. Procédé pour fabriquer des bandes d'acier au carbone et d'acier faiblement allié ayant une microstructure fortement contrôlée, comportant, à la suite, les étapes suivantes consistant à :
■ couler, dans une machine de coulée continue à deux rouleaux (A), des bandes ayant une épaisseur dans la plage de 1 à 6 mm et une composition, exprimée en pourcentage en masse, comportant les composants suivants :
0,02 à 0,20 C, 0,1 à 1,6 Mn, 0,02 à 2,00 Si, < 0,05 Al, < 0,03 S, < 0,1 P, 0,01 à 1,5 Cr, 0,01 à 0,5 Ni, < 0,5 Mo, 0,003 à 0,012 N, et, de manière facultative, < 0,03 Ti, < 0,10 V, < 0,035 Nb, < 0,005 B, le reste étant Fe et des impuretés inévitables,
■ refroidir de manière commandée la bande dans la section comprise entre les rouleaux de coulée et un système de roulage (E),
■ déformer à chaud la bande coulée par ledit système de roulage (E) à une température dans la plage de 1150 à (Ar₁ - 100)°C, jusqu'à effectuer une réduction d'épaisseur de 15 à 80 % de celle-ci, ladite déformation à chaud étant sélectionnée parmi le groupe constitué de :
- roulage à des températures > Ar₃ et dans une phase complètement austénitique, Ar₃ étant la température de début de transformation de l'austénite refroidie en continu,
- roulage, à une température < Ar₁ et dans une phase complètement ferritique,
- roulage, à des températures dans la plage de Ar₃ à Ar₁ et sous des conditions de co-existence de la phase austénitique et de la phase ferritique,
■ maintenir la bande à une température commandée dans un système isolé (F) compris entre une sortie du système de roulage (E) et une entrée du système de chauffage (G),
■ chauffer la bande à l'aide du système de chauffage (G) à des températures dans la plage de 670 à 1150°C pendant des périodes dans la plage de 5 à 40 s, de manière à obtenir une recristallisation de bande en volume > 95 %,
■ refroidir de manière commandée la section comprise entre une sortie dudit système de chauffage (G) et un système d'emballage, de manière facultative ayant plusieurs bobines (N, P), de la bande ainsi obtenue.

2. Procédé pour fabriquer des bandes d'acier au carbone et d'acier faiblement allié selon la revendication 1, dans lequel, au cours de ladite étape de coulée, la composition de ladite bande comporte également : < 0,03 Ti, < 0,10 V, < 0,035 Nb et < 0,005 B.

3. Procédé pour fabriquer des bandes d'acier au carbone et d'acier faiblement allié selon la revendication 1 ou 2, dans lequel ledit refroidissement commandé de la section comprise entre les rouleaux de coulée et les rouleaux pinceurs C, et entre les rouleaux pinceurs (C) et le système de roulage (E) a lieu par l'intermédiaire d'une paire de systèmes (B et D), ayant des modules, individuellement actionnables, variables dans les sections individuelles et capables d'imprimer sur la bande des vitesses de refroidissement allant jusqu'à 200°C/s.

4. Procédé pour fabriquer des bandes d'acier au carbone et d'acier faiblement allié selon la revendication 3, dans lequel ledit refroidissement est obtenu à l'aide de modes de refroidissement sélectionnés parmi le groupe comportant : de l'air naturel, de l'air forcé, des jets de gaz inerte dans une chambre rendue inerte, de l'air-eau, de l'eau et des combinaisons de ceux-ci.

5. Procédé pour fabriquer des bandes d'acier au carbone et d'acier faiblement allié selon l'une quelconque des revendications 1 à 4, dans lequel ledit système de chauffage (G) fonctionne sous une atmosphère réductrice ou non-oxydante.

6. Procédé pour fabriquer des bandes d'acier au carbone et d'acier faiblement allié selon la revendication 5, dans lequel ledit système de chauffage (G) fonctionne à des températures sélectionnées parmi le groupe comportant : des températures correspondant à celle de l'existence de la seule phase austénitique, des températures correspondant à celle de l'existence de la seule phase ferritique, des températures correspondant à celle de la co-existence des phases ferritique et austénitique.

7. Procédé pour fabriquer des bandes d'acier au carbone et d'acier faiblement allié selon la revendication 6, dans lequel ledit système de chauffage (G) est suivi d'un système (H) pour nettoyer la surface de bande et pour éliminer à partir de celle-ci des oxydes ou résidus d'oxyde réduits partiellement ou totalement par l'atmosphère du four.

8. Procédé pour fabriquer des bandes d'acier au carbone et d'acier faiblement allié selon l'une quelconque des revendications 1 à 7, dans lequel la bande est maintenue à une température commandée sur la sortie du système de roulage (E) par un système (F) comportant un tunnel isolé contenant de l'air, ou un gaz inerte, ou des combinaisons de ceux-ci.

9. Procédé pour fabriquer des bandes d'acier au carbone et d'acier faiblement allié selon l'une quelconque des revendications 1 à 8, dans lequel, sur la sortie du système de chauffage (G), la bande est soumise à un refroidissement à l'aide d'au moins trois modules (I, L, M), positionnés le long d'un trajet de rouleau, capables d'imprimer sur la bande des vitesses de refroidissement variables dans les sections individuelles et se trouvant dans la plage de 800°C/s à 0,01°C/s.

10. Procédé pour fabriquer des bandes d'acier au carbone et d'acier faiblement allié selon la revendication 9, dans lequel dans un desdits au moins trois modules (I, L, M), une galvanisation de bande peut être effectuée.

11. Procédé pour fabriquer des bandes d'acier au carbone et d'acier faiblement allié selon l'une quelconque des revendications précédentes, dans lequel la déformation à chaud de la bande coulée a lieu par l'intermédiaire de deux montants consécutifs, chacun fournissant une réduction d'épaisseur de 15 à 40 %.

12. Procédé pour fabriquer des bandes d'acier au carbone et d'acier faiblement allié selon la revendication 11, dans lequel le temps de passage entre des montants consécutifs est plus court que le temps nécessaire pour obtenir 50 % de recristallisation en volume.

13. Procédé pour fabriquer des bandes d'acier au carbone et d'acier faiblement allié selon la revendication 3, dans lequel on a agencé un système (R) pour chauffer la bande dans la section comprise entre les rouleaux pinceurs (C) et le système de roulage (E).

14. Procédé pour fabriquer des bandes d'acier au carbone et d'acier faiblement allié selon la revendication 13, dans lequel ledit système de chauffage (R) est positionné en aval du système de refroidissement commandé (D).

15. Procédé pour fabriquer des bandes d'acier au carbone et d'acier faiblement allié selon l'une quelconque des revendications précédentes, dans lequel la bande est emballée à des températures dans la plage de 150 à 900°C.
